



US011873587B2

(12) **United States Patent**  
Adams et al.

(10) **Patent No.:** US 11,873,587 B2  
(45) **Date of Patent:** Jan. 16, 2024

(54) **FLAME RESISTANT FABRICS**(71) Applicant: **Southern Mills, Inc.**, Union City, GA (US)(72) Inventors: **Dominique Janay Adams**, Fairburn, GA (US); **Charles S. Dunn**, Griffin, GA (US); **Elijah Dufty**, Atlanta, GA (US); **Michael T. Stanhope**, Atlanta, GA (US)(73) Assignee: **Southern Mills, Inc.**, Union City, GA (US)

(\*) Notice: Subject to any disclaimer, the term of this patent is extended or adjusted under 35 U.S.C. 154(b) by 436 days.

(21) Appl. No.: 17/175,647

(22) Filed: Feb. 13, 2021

(65) **Prior Publication Data**

US 2021/0164133 A1 Jun. 3, 2021

**Related U.S. Application Data**

(62) Division of application No. 16/832,991, filed on Mar. 27, 2020.

(60) Provisional application No. 62/825,350, filed on Mar. 28, 2019.

(51) **Int. Cl.****D02G 3/44** (2006.01)**D03D 15/513** (2021.01)(52) **U.S. Cl.**CPC ..... **D02G 3/443** (2013.01); **D03D 15/513** (2021.01); **D10B 2201/20** (2013.01); **D10B 2321/101** (2013.01); **D10B 2331/021** (2013.01); **Y10T 442/3984** (2015.04)(58) **Field of Classification Search**

None

See application file for complete search history.

(56) **References Cited**

## U.S. PATENT DOCUMENTS

|             |         |                     |
|-------------|---------|---------------------|
| 2,333,824 A | 11/1943 | Schoepf             |
| 2,696,723 A | 12/1954 | Frith, Jr.          |
| 3,097,442 A | 7/1963  | Willingham, Jr.     |
| 3,729,920 A | 5/1973  | Sayers et al.       |
| 3,763,644 A | 10/1973 | Jackson, Jr. et al. |
| 3,806,959 A | 4/1974  | Gross               |
| 3,918,901 A | 11/1975 | Ida et al.          |
| 4,533,592 A | 8/1985  | Bingham             |
| 4,615,934 A | 10/1986 | Ellison             |
| 4,668,234 A | 5/1987  | Vance et al.        |
| 4,705,523 A | 11/1987 | Hussamy             |
| 4,705,527 A | 11/1987 | Hussamy             |
| 4,710,200 A | 12/1987 | Cates et al.        |
| 4,741,740 A | 5/1988  | Davis et al.        |
| 4,752,300 A | 6/1988  | Johnson             |
| 4,759,770 A | 7/1988  | Cates et al.        |
| 4,814,222 A | 3/1989  | Davis et al.        |
| 4,868,041 A | 9/1989  | Yamagishi et al.    |
| 4,898,596 A | 2/1990  | Riggins et al.      |

|             |         |                  |
|-------------|---------|------------------|
| 4,902,300 A | 2/1990  | Johnson et al.   |
| 4,920,000 A | 4/1990  | Green            |
| 4,970,255 A | 11/1990 | Reimann et al.   |
| 4,981,488 A | 1/1991  | Cates et al.     |
| 4,996,099 A | 2/1991  | Cooke et al.     |
| 5,043,207 A | 8/1991  | Donovan et al.   |
| 5,074,889 A | 12/1991 | Hodge et al.     |
| 5,141,542 A | 8/1992  | Fangeat et al.   |
| 5,150,476 A | 9/1992  | Statham et al.   |
| 5,174,790 A | 12/1992 | Riggins et al.   |
| 5,208,105 A | 5/1993  | Ichibori et al.  |
| 5,215,545 A | 6/1993  | Cates et al.     |
| 5,275,627 A | 1/1994  | Cates et al.     |
| 5,306,312 A | 4/1994  | Riggins et al.   |
| 5,323,815 A | 6/1994  | Barbeau et al.   |
| 5,356,700 A | 10/1994 | Tanaka et al.    |
| 5,447,540 A | 9/1995  | Kobayashi et al. |
| 5,456,728 A | 10/1995 | Schwarz et al.   |
| 5,466,265 A | 11/1995 | Riegels et al.   |

(Continued)

## FOREIGN PATENT DOCUMENTS

|    |               |        |
|----|---------------|--------|
| AU | 2005200963 A1 | 3/2005 |
| AU | 2007290499 B2 | 7/2012 |

(Continued)

## OTHER PUBLICATIONS

PCT Patent Application No. PCT/US2020/025434, International Search Report and Written Opinion, dated Aug. 17, 2020, 15 pages. Restriction Requirement, U.S. Appl. No. 16/832,991, dated Dec. 14, 2020, 5 pages.

U.S. Appl. No. 16/832,991, Non-Final Office Action, dated Jun. 7, 2022, 15 pages.

Office Action, Japanese Patent Application No. 2021-557646, Office Action, dated Apr. 12, 2022, 4 pages.

Office Action, Chinese Patent Application No. 202080039337.7, dated Nov. 21, 2022, 26 pages.

(Continued)

Primary Examiner — Jenna L Johnson

(74) Attorney, Agent, or Firm — Kilpatrick Townsend &amp; Stockton LLP

(57) **ABSTRACT**

Embodiments of the present invention relate to flame resistant fabrics formed with inherently flame resistant fibers that provide the requisite thermal and arc protection, that have improved comfort, and that, in some embodiments, are less expensive than other fabrics formed with inherently flame resistant fibers. Improved comfort and lower cost can be achieved by predominantly locating the inherently flame resistant fibers on the front face of the fabric to impart the requisite thermal and arc protection and predominantly locating the more comfortable (and less expensive) fibers on the back face of the fabric positioned next to the wearer. In this way, overall protection of the fabric is maintained while improving comfort. Some embodiments of such fabrics may also achieve NFPA 70E PPE Category 2 protection.

| (56)                  | References Cited |                       |                  |         |                           |
|-----------------------|------------------|-----------------------|------------------|---------|---------------------------|
| U.S. PATENT DOCUMENTS |                  |                       |                  |         |                           |
| 5,488,101 A           | 1/1996           | Ogino et al.          | 9,034,777 B2     | 5/2015  | Hines et al.              |
| 5,514,457 A           | 5/1996           | Fels et al.           | 9,259,599 B2     | 2/2016  | Stanhope et al.           |
| 5,527,597 A           | 6/1996           | Stanhope et al.       | 9,370,212 B2     | 6/2016  | Zhu                       |
| 5,539,928 A           | 7/1996           | Aldridge              | 9,683,315 B2     | 6/2017  | Schmitt et al.            |
| 5,578,368 A           | 11/1996          | Forsten et al.        | 9,706,804 B1     | 7/2017  | Emery et al.              |
| 5,609,950 A           | 3/1997           | Kampl et al.          | 9,765,454 B2     | 9/2017  | Tutterow et al.           |
| 5,640,718 A           | 6/1997           | Aldridge              | 9,878,185 B2     | 1/2018  | Underwood et al.          |
| 5,685,015 A           | 11/1997          | Aldridge              | 9,938,645 B2     | 4/2018  | Stanhope et al.           |
| 5,694,981 A           | 12/1997          | Stanhope et al.       | 9,988,745 B2     | 6/2018  | Sanchez et al.            |
| 5,724,673 A           | 3/1998           | Aldridge              | 10,030,326 B2    | 7/2018  | Hines, Jr. et al.         |
| 5,727,401 A           | 3/1998           | Statham               | 10,072,365 B2    | 9/2018  | Birk et al.               |
| 5,776,746 A           | 7/1998           | Denney, Jr.           | 10,101,128 B2    | 10/2018 | Cushingham et al.         |
| 5,819,316 A           | 10/1998          | Aldridge              | 10,183,465 B1    | 1/2019  | Bowman et al.             |
| 5,824,614 A           | 10/1998          | Gadoury               | 10,316,440 B2    | 6/2019  | Stanhope et al.           |
| 5,830,574 A           | 11/1998          | Gadoury               | 10,385,481 B2    | 8/2019  | Underwood et al.          |
| 5,849,648 A           | 12/1998          | Kent et al.           | 10,422,055 B2    | 9/2019  | Sytz                      |
| 5,858,888 A           | 1/1999           | Underwood et al.      | 10,485,281 B2    | 11/2019 | Stanhope et al.           |
| 5,885,307 A           | 3/1999           | Gadoury               | 10,487,424 B2    | 11/2019 | Stanhope et al.           |
| 5,891,813 A           | 4/1999           | Gadoury               | 10,640,893 B2    | 5/2020  | Sarzotti et al.           |
| 5,906,891 A           | 5/1999           | Shida et al.          | 10,704,169 B2    | 7/2020  | Habicht et al.            |
| 5,920,905 A           | 7/1999           | Aldridge              | 10,774,451 B2    | 9/2020  | Stanhope et al.           |
| 5,928,971 A           | 7/1999           | Ellis et al.          | 10,870,932 B2    | 12/2020 | Stanhope et al.           |
| 6,132,476 A           | 10/2000          | Lunsford et al.       | 11,306,418 B2    | 4/2022  | Stanhope et al.           |
| 6,146,759 A           | 11/2000          | Land                  | 11,421,348 B2    | 8/2022  | Stanhope et al.           |
| 6,184,282 B1          | 2/2001           | Gareiss et al.        | 2001/0009832 A1  | 7/2001  | Shaffer et al.            |
| 6,192,520 B1          | 2/2001           | Underwood et al.      | 2002/0016985 A1  | 2/2002  | Kelleher et al.           |
| 6,225,383 B1          | 5/2001           | Hirono et al.         | 2002/0064654 A1  | 5/2002  | Luo et al.                |
| 6,247,179 B1          | 6/2001           | Underwood et al.      | 2002/0069453 A1  | 6/2002  | Kelleher et al.           |
| 6,255,371 B1          | 7/2001           | Schlosser et al.      | 2002/0182967 A1  | 12/2002 | Erb, Jr. et al.           |
| 6,342,548 B2          | 1/2002           | Flippo et al.         | 2003/0082972 A1  | 5/2003  | Monfalcone, III et al.    |
| 6,410,140 B1          | 6/2002           | Land et al.           | 2003/0098068 A1  | 5/2003  | Chi et al.                |
| 6,430,754 B1          | 8/2002           | Taylor et al.         | 2003/0148689 A1  | 8/2003  | Lapiere                   |
| 6,451,070 B1          | 9/2002           | Kent et al.           | 2003/0167580 A1  | 9/2003  | Lunsford et al.           |
| 6,534,175 B1          | 3/2003           | Zhu et al.            | 2003/0226612 A1  | 12/2003 | Zhu et al.                |
| 6,547,835 B1          | 4/2003           | Lunsford et al.       | 2003/0228812 A1  | 12/2003 | Stanhope et al.           |
| 6,626,964 B1          | 9/2003           | Lunsford et al.       | 2003/0228821 A1  | 12/2003 | Zhu et al.                |
| 6,668,868 B2          | 12/2003          | Howland et al.        | 2003/0232560 A1  | 12/2003 | Corner                    |
| 6,693,052 B2          | 2/2004           | Howland               | 2004/0001978 A1  | 1/2004  | Bader et al.              |
| 6,706,650 B2          | 3/2004           | Gibson et al.         | 2004/0029473 A1  | 2/2004  | McKee et al.              |
| 6,735,789 B2          | 5/2004           | Kelleher et al.       | 2004/0045103 A1  | 3/2004  | Lunsford et al.           |
| 6,787,228 B2          | 9/2004           | Campbell et al.       | 2004/0065072 A1  | 4/2004  | Zhu et al.                |
| 6,818,024 B2          | 11/2004          | Lunsford et al.       | 2004/0076824 A1  | 4/2004  | Urabe et al.              |
| 6,840,288 B2          | 1/2005           | Zhu et al.            | 2004/0152378 A1  | 8/2004  | Stanhope et al.           |
| 6,861,378 B2          | 3/2005           | Cunningham et al.     | 2004/0192134 A1  | 9/2004  | Gibson et al.             |
| 6,867,154 B1          | 3/2005           | Lunsford et al.       | 2005/0025962 A1  | 2/2005  | Zhu et al.                |
| 6,946,412 B2          | 9/2005           | Campbell et al.       | 2005/0025963 A1  | 2/2005  | Zhu                       |
| 6,974,785 B1          | 12/2005          | Barbeau et al.        | 2005/0032449 A1  | 2/2005  | Lovasic et al.            |
| 7,013,496 B2          | 3/2006           | Dunn                  | 2005/0050619 A1  | 3/2005  | Dunn                      |
| 7,065,950 B2          | 6/2006           | Zhu et al.            | 2005/0060820 A1  | 3/2005  | Lunsford et al.           |
| 7,073,538 B2          | 7/2006           | Bhatnagar et al.      | 2005/0064020 A1  | 3/2005  | Schuette et al.           |
| 7,156,883 B2          | 1/2007           | Lovasic et al.        | 2005/0119379 A1  | 6/2005  | Martens et al.            |
| 7,284,398 B2          | 10/2007          | Hubner                | 2005/0197028 A1  | 9/2005  | Hartgrove et al.          |
| 7,393,800 B2          | 7/2008           | Corner                | 2005/0208855 A1  | 9/2005  | Zhu                       |
| 7,402,538 B2          | 7/2008           | Bader et al.          | 2005/0245163 A1  | 11/2005 | Aneja et al.              |
| 7,473,659 B2          | 1/2009           | Sytz                  | 2005/0287364 A1  | 12/2005 | Zhu et al.                |
| 7,589,036 B2          | 9/2009           | Corner et al.         | 2006/0030228 A1  | 2/2006  | Truesdale, III            |
| 7,634,819 B2          | 12/2009          | Grey                  | 2006/0040575 A1  | 2/2006  | Kelleher et al.           |
| 7,676,855 B2          | 3/2010           | Dunn                  | 2006/0068664 A1  | 3/2006  | Gibson et al.             |
| 7,681,417 B2          | 3/2010           | Haghara et al.        | 2006/0084337 A1  | 4/2006  | Corner et al.             |
| 7,703,405 B2          | 4/2010           | Bridgeman et al.      | 2006/0116043 A1  | 6/2006  | Hope et al.               |
| 7,854,017 B2          | 12/2010          | Laton                 | 2006/0143809 A1  | 7/2006  | Dunn                      |
| 7,862,865 B2          | 1/2011           | Truesdale, III et al. | 2006/0264136 A1  | 11/2006 | Chiantese                 |
| RE42,209 E            | 3/2011           | Lunsford et al.       | 2007/0178788 A1  | 8/2007  | Day et al.                |
| 8,017,532 B2          | 9/2011           | Okada                 | 2007/0184737 A1  | 12/2006 | Ashley et al.             |
| 8,071,492 B2          | 12/2011          | Hess et al.           | 2007/026752 A1   | 2/2007  | Thiriot et al.            |
| 8,133,584 B2          | 3/2012           | Zhu                   | 2007/0123127 A1  | 5/2007  | Hirschmann, Jr. et al.    |
| 8,327,469 B2          | 12/2012          | Curtis                | 2007/0148455 A1  | 6/2007  | Ke                        |
| 8,347,420 B2          | 1/2013           | Kruszewski et al.     | 2007/0249247 A1  | 10/2007 | Truesdale, III et al.     |
| 8,528,120 B2          | 9/2013           | Underwood et al.      | 2007/0249250 A1  | 10/2007 | Servajeian                |
| 8,536,076 B1          | 9/2013           | Byles                 | 2008/0057807 A1* | 3/2008  | Tutterow ..... A41D 31/08 |
| 8,614,156 B2          | 12/2013          | Hess et al.           |                  |         | 428/221                   |
| 8,652,975 B1          | 2/2014           | Atkinson et al.       | 2008/0086798 A1  | 4/2008  | Allen, II et al.          |
| 8,703,631 B2          | 4/2014           | Sytz                  | 2008/0139752 A1  | 6/2008  | De et al.                 |
| 8,741,789 B2          | 6/2014           | Li et al.             | 2008/0148468 A1  | 6/2008  | Laton et al.              |
| 8,898,821 B2          | 12/2014          | Stanhope et al.       | 2008/0152888 A1  | 6/2008  | Tutterow et al.           |
|                       |                  |                       | 2008/0182470 A1  | 7/2008  | Fang et al.               |

(56)

## References Cited

## FOREIGN PATENT DOCUMENTS

| U.S. PATENT DOCUMENTS |         |                       | BE                     | 1015931         | 11/2005     |        |
|-----------------------|---------|-----------------------|------------------------|-----------------|-------------|--------|
| 2008/0227352 A1       | 9/2008  | Byles et al.          | CA                     | 2078626 C       | 4/1999      |        |
| 2008/0295232 A1       | 12/2008 | Truesdale, III et al. | CN                     | 1172508 A       | 2/1998      |        |
| 2009/0030111 A1       | 1/2009  | Barnes et al.         | CN                     | 1201474 A       | 12/1998     |        |
| 2009/0139016 A1       | 6/2009  | Zhu et al.            | CN                     | 1575359 A       | 2/2005      |        |
| 2009/0178186 A1       | 7/2009  | Truesdale             | CN                     | 1950455 A       | 4/2007      |        |
| 2009/0226653 A1       | 9/2009  | Harris et al.         | CN                     | 101166852 A     | 4/2008      |        |
| 2009/0255038 A1       | 10/2009 | Curtis                | CN                     | 101263253 A     | 9/2008      |        |
| 2010/0009186 A1       | 1/2010  | Zhu                   | CN                     | 101326315 A     | 12/2008     |        |
| 2010/0024103 A1       | 2/2010  | Kelleher et al.       | CN                     | 101611182 A     | 12/2009     |        |
| 2010/0075557 A1       | 3/2010  | Shteiyer              | CN                     | 101657573 A     | 2/2010      |        |
| 2010/0112312 A1       | 5/2010  | Tutterow et al.       | CN                     | 101754998 A     | 6/2010      |        |
| 2010/0143683 A1       | 6/2010  | Chiou                 | CN                     | 102859055 A     | 1/2013      |        |
| 2010/0210162 A1       | 8/2010  | Li et al.             | CN                     | 102995224 A     | 3/2013      |        |
| 2010/0297905 A1*      | 11/2010 | Ulrich .....          | D03D 15/513<br>442/302 | CN              | 103221597 A | 7/2013 |
|                       |         |                       |                        | CN              | 103603123 A | 2/2014 |
|                       |         |                       |                        | CN              | 103857837 A | 6/2014 |
| 2010/0299816 A1       | 12/2010 | Zhu                   | CN                     | 104685118 A     | 6/2015      |        |
| 2010/0299817 A1       | 12/2010 | Zhu                   | CN                     | 105220314 B     | 3/2017      |        |
| 2011/0010827 A1*      | 1/2011  | Stanhope .....        | D02G 3/443<br>2/81     | CN              | 107034574 A | 8/2017 |
|                       |         |                       |                        | CN              | 107075752 A | 8/2017 |
| 2011/0023206 A1       | 2/2011  | Dunn et al.           | CN                     | 108474147 A     | 8/2018      |        |
| 2011/0138523 A1       | 6/2011  | Layson, Jr. et al.    | DE                     | 202004005008 U1 | 6/2004      |        |
| 2011/0159364 A1       | 6/2011  | Nishinaka et al.      | DE                     | 202010011193 U1 | 12/2010     |        |
| 2011/0250810 A1       | 10/2011 | Zhu                   | EP                     | 0330163 A2      | 8/1989      |        |
| 2011/0275263 A1       | 11/2011 | Li et al.             | EP                     | 0364194 A2      | 4/1990      |        |
| 2011/0281097 A1       | 11/2011 | Li et al.             | EP                     | 0559128 A1      | 9/1993      |        |
| 2012/0031783 A1       | 2/2012  | Fay, III et al.       | EP                     | 0412195 B1      | 6/1995      |        |
| 2012/0090080 A1       | 4/2012  | Stanhope et al.       | EP                     | 1247885         | 10/2002     |        |
| 2012/0102632 A1       | 5/2012  | Zhu                   | EP                     | 1754813 A1      | 2/2007      |        |
| 2012/0122361 A1       | 5/2012  | Hand et al.           | EP                     | 1767677 A1      | 3/2007      |        |
| 2012/0159697 A1       | 6/2012  | Zhu                   | EP                     | 2096199 A1      | 9/2009      |        |
| 2012/0171918 A1       | 7/2012  | Lawson, III et al.    | EP                     | 1498522 B1      | 9/2010      |        |
| 2012/0183747 A1       | 7/2012  | Bader et al.          | EP                     | 2567945 A2      | 3/2013      |        |
| 2012/0210481 A1       | 8/2012  | Rock et al.           | EP                     | 2738294 A1      | 6/2014      |        |
| 2012/0244772 A1       | 9/2012  | Elder                 | EP                     | 3425093 A1      | 1/2019      |        |
| 2012/0270456 A1       | 10/2012 | Gstettner et al.      | FR                     | 3831992 B1      | 1/2022      |        |
| 2012/0286177 A1       | 11/2012 | Cliver et al.         | FR                     | 2514934 A1      | 4/1983      |        |
| 2013/0008554 A1       | 1/2013  | Fisher et al.         | FR                     | 2691721 A1      | 12/1993     |        |
| 2013/0055490 A1       | 3/2013  | Zhu                   | FR                     | 2836932 A1      | 9/2003      |        |
| 2013/0055491 A1       | 3/2013  | Zhu                   | GB                     | 1126432         | 9/1968      |        |
| 2013/0065470 A1       | 3/2013  | Rock et al.           | GB                     | 2025789 A       | 1/1980      |        |
| 2013/0149932 A1       | 6/2013  | Leitner et al.        | JP                     | H01-221537 A    | 9/1989      |        |
| 2013/0212790 A1       | 8/2013  | Waxman et al.         | JP                     | 02127466 A      | 5/1990      |        |
| 2013/0216810 A1       | 8/2013  | Hines et al.          | JP                     | 04501221 A      | 3/1992      |        |
| 2013/0244527 A1       | 9/2013  | Sarzotti et al.       | JP                     | H08158201 A     | 6/1996      |        |
| 2014/0026303 A1       | 1/2014  | Zhu                   | JP                     | H08209486 A     | 8/1996      |        |
| 2014/0187113 A1       | 7/2014  | Hines, Jr. et al.     | JP                     | H08-260286 A    | 10/1996     |        |
| 2014/0208491 A1       | 7/2014  | Schmitt et al.        | JP                     | 2703390 B2      | 1/1998      |        |
| 2014/0261852 A1       | 9/2014  | Bonner et al.         | JP                     | 1088448 A       | 4/1998      |        |
| 2015/0086758 A1       | 3/2015  | Tutterow et al.       | JP                     | 10280230 A      | 10/1998     |        |
| 2015/0297919 A1       | 10/2015 | Stanhope et al.       | JP                     | 2000-303257 A   | 10/2000     |        |
| 2015/0322598 A1       | 11/2015 | Stanhope et al.       | JP                     | 2000-328363 A   | 11/2000     |        |
| 2015/0361599 A1       | 12/2015 | Minor                 | JP                     | 2001-234066 A   | 8/2001      |        |
| 2016/0201236 A1       | 7/2016  | Matsumoto et al.      | JP                     | 2003-105659 A   | 4/2003      |        |
| 2016/0362831 A1       | 12/2016 | Minor                 | JP                     | 2005-532484 A   | 10/2005     |        |
| 2017/0175302 A1       | 6/2017  | Habicht et al.        | JP                     | 2007-500802 A   | 1/2007      |        |
| 2017/0203540 A1       | 7/2017  | Colatruglio et al.    | JP                     | 2007-500803 A   | 1/2007      |        |
| 2017/0295875 A1       | 10/2017 | Ohzeki et al.         | JP                     | 2007-507595 A   | 3/2007      |        |
| 2017/0370032 A1       | 12/2017 | Stanhope et al.       | JP                     | 2008-031618 A   | 2/2008      |        |
| 2018/0002840 A1       | 1/2018  | Tutterow et al.       | JP                     | 2008208509 A    | 9/2008      |        |
| 2018/0030627 A1       | 2/2018  | Stanhope et al.       | JP                     | 2011-502218 A   | 1/2011      |        |
| 2018/0127899 A1       | 5/2018  | Tutterow et al.       | JP                     | 5090778 B2      | 9/2012      |        |
| 2018/0171516 A1       | 6/2018  | Stanhope et al.       | JP                     | 2013-542334 A   | 11/2013     |        |
| 2018/0245251 A1       | 8/2018  | Dash et al.           | JP                     | 5887366 B2      | 2/2016      |        |
| 2018/0274136 A1       | 9/2018  | Guo et al.            | JP                     | 5887376 B2      | 2/2016      |        |
| 2018/0313006 A1       | 11/2018 | Stanhope et al.       | JP                     | 930009831       | 10/1993     |        |
| 2018/0371647 A1       | 12/2018 | Sato et al.           | KR                     | 1020060122840 A | 11/2006     |        |
| 2019/0242038 A1       | 8/2019  | Stanhope et al.       | KR                     | 1020070012391 A | 1/2007      |        |
| 2019/0301059 A1       | 10/2019 | Flack et al.          | RU                     | 2402648 C1      | 10/2010     |        |
| 2019/0309451 A1       | 10/2019 | King et al.           | TW                     | 200538499 A     | 12/2005     |        |
| 2020/0308735 A1       | 10/2020 | Adams et al.          | TW                     | 200613448 A     | 5/2006      |        |
| 2021/0292936 A1       | 9/2021  | Ringo                 | TW                     | 200617097 A     | 6/2006      |        |
|                       |         |                       | WO                     | 93/24690 A1     | 12/1993     |        |
|                       |         |                       | WO                     | 0000686 A1      | 1/2000      |        |
|                       |         |                       | WO                     | 0220887 A2      | 3/2002      |        |

(56)

**References Cited**

## FOREIGN PATENT DOCUMENTS

WO 02052077 A2 7/2002  
WO 2004/005606 A1 1/2004  
WO 2004002254 A1 1/2004  
WO 2004088023 10/2004  
WO 2005/033192 A1 4/2005  
WO 2005/090660 A1 9/2005  
WO 2005/095685 A1 10/2005  
WO 2005092132 A1 10/2005  
WO 2006008900 A1 1/2006  
WO 2006017709 2/2006  
WO 2006034131 A2 3/2006  
WO 2006043958 A1 4/2006  
WO 2006049626 A1 5/2006  
WO 2006101933 A2 9/2006  
WO 2007061423 A2 5/2007  
WO 2007070079 A1 6/2007  
WO 2007133177 A2 11/2007  
WO 2008/027454 A1 3/2008  
WO 2008048308 A2 4/2008  
WO 2009/101930 A1 8/2009  
WO 2010091476 A1 8/2010  
WO 2010/135423 A1 11/2010  
WO 2011/056467 A2 5/2011  
WO 2012/040332 A2 3/2012  
WO 2012/077681 A1 6/2012  
WO 2012/121759 A2 9/2012  
WO 2013/074181 A2 5/2013  
WO 2016/010659 A1 1/2016  
WO 2016/033593 A1 3/2016  
WO 2017/070529 A1 4/2017

## OTHER PUBLICATIONS

“Fabric Flame Retardant Treatment “Precondensate”/NH3 Process”, Technical Bulletin, Cotton Incorporated, TRI 4002, 2003, 12 pages.

“GlenGuard™ FR”, Glen Raven Technical Fabrics, LLC, 4 pages.  
“Pigments as Colorants: Pigmenting or Pigmentation”, Textile Dyeing and Coloration, Chapter 23, 1997, 12 pages.  
“Polyesters and Polyamides”, Conclusions and future Trends, Woodhead Publishing Limited, Woodhead Publishing in Textiles, No. 71, 2008, p. 320.  
Horrocks et al., “Fabric Flame Retardant Treatment”, Fire Retardant Materials, vol. 148, 2003, 12 pages.  
Mathur et al., “Color and Weave Relationship in Woven Fabrics”, Advances in Modern Woven Fabrics Technology, IntechOpen, Jul. 27, 2011, 24 pages.  
Yang et al., “A Durable Flame Retardant for Cellulosic Fabrics”, Polymer degradation and stability, vol. 97, No. 11, Nov. 1, 2012, pp. 2467-2472.  
“Introducing Our Lightest Dual Hazard Fabric Ever”, DRIFIRE, Product Line, 2015, 3 pages.  
“Ready for Action”, Lion, Dec. 21, 2011, 60 pages.  
“Tools & Technologies: Fire Service Prepares for Change in PPE Technology”, Trade Journal, Firehouse, vol. 37, Feb. 1, 2012, 3 pages.  
U.S. Appl. No. 16/832,991, Final Office Action, dated Jul. 27, 2021, 13 pages.  
U.S. Appl. No. 16/832,991, Non-Final Office Action, dated Feb. 26, 2021, 8 pages.  
PCT Patent Application No. PCT/US2020/025434, International Preliminary Report on Patentability, dated Oct. 7, 2021, 10 pages.  
Smith , “Lyocell—One Fiber, Many Faces”, Ohio State University, Available Online at: <http://web.archive.org/web/20060830212533/http://ohioline.osu.edu/hyg-fact/5000/5572.html>, Aug. 30, 2016, pp. 1-5.  
Australian Patent Application No. 2020245599, First Examination Report, dated Nov. 18, 2021, 4 pages.  
Canadian Patent Application No. 3,135,175, Office Action, dated Nov. 22, 2021, 4 pages.  
New Zealand Patent Application No. 781462, First Examination Report, dated Nov. 17, 2021, 1 page.

\* cited by examiner

## FLAME RESISTANT FABRICS

## CROSS-REFERENCE TO RELATED APPLICATIONS

This application is a divisional of U.S. patent application Ser. No. 16/832,991, filed Mar. 27, 2020 and entitled "Flame Resistant Fabrics", which claims the benefit of U.S. Provisional Application No. 62/825,350, filed Mar. 28, 2019 and entitled "Low Cost Flame Resistant Fabrics with Inherently Flame Resistant Fibers," the entirety of all which are hereby incorporated by reference.

## FIELD OF THE INVENTION

Embodiments of the present invention relates to low cost and low weight flame resistant protective fabrics and garments made therefrom that impart improved protection to the wearer.

## BACKGROUND

Many occupations can potentially expose an individual to electrical arc flash and/or flames. Workers who may be exposed to accidental electric arc flash and/or flames risk serious burn injury unless they are properly protected. To avoid being injured while working in such conditions, these individuals typically wear protective garments constructed of flame resistant materials designed to protect them from electrical arc flash and/or flames. Such protective clothing can include various garments, for example, coveralls, pants, and shirts. Standards have been promulgated that govern the performance of such garments (or constituent layers or parts of such garments) to ensure that the garments sufficiently protect the wearer in hazardous situations. Fabrics from which such garments are constructed, and consequently the resulting garments as well, are required to pass a variety of safety and/or performance standards, including ASTM F1506, NFPA 70E, NFPA 2112, and NFPA 1975.

ASTM F1506 (Standard Performance Specification for Flame Resistant and Arc Rated Textile Materials for Wearing Apparel for Use by Electrical Workers Exposed to Momentary Electric Arc and Related Thermal Hazards, 2018 edition, incorporated herein by reference) requires arc rating testing of protective fabrics worn by electrical workers. The arc rating value represents a fabric's performance when exposed to an electrical arc discharge. The arc rating is expressed in  $\text{cal}/\text{cm}^2$  (calories per square centimeter) and is derived from the determined value of the arc thermal performance value (ATPV) or Energy Breakopen threshold ( $E_{BT}$ ). ATPV is defined as the arc incident energy on a material that results in a 50% probability that sufficient heat transfer through the specimen is predicted to cause the onset of second-degree burn injury based on the Stoll Curve.  $E_{BT}$  is the arc incident energy on a material that results in a 50% probability of breakopen. Breakopen is defined as any open area in the material at least  $1.6 \text{ cm}^2$  ( $0.5 \text{ in.}^2$ ). The arc rating of a material is reported as either ATPV or  $E_{BT}$ , whichever is the lower value. The ATPV and  $E_{BT}$  is determined pursuant to the testing methodology set forth in ASTM F1959 (Standard Test Method for Determining the Arc Rating of Materials for Clothing, 2014 edition, incorporated herein by reference), where sensors measure thermal energy properties of protective fabric specimens during exposure to a series of electric arcs.

NFPA 70E (Standard for Electrical Safety in the Workplace, 2018 edition, incorporated herein by reference) offers

a method to match protective clothing to potential exposure levels incorporating Personal Protective Equipment (PPE) Categories. Protective fabrics are tested to determine their arc rating, and the measured arc rating determines the PPE Category for a fabric as follows:

- PPE Category and ATPV
- PPE Category 1:  $\text{ATPV}/E_{BT}$ :  $4 \text{ cal}/\text{cm}^2$
- PPE Category 2:  $\text{ATPV}/E_{BT}$ :  $8 \text{ cal}/\text{cm}^2$
- PPE Category 3:  $\text{ATPV}/E_{BT}$ :  $25 \text{ cal}/\text{cm}^2$
- PPE Category 4:  $\text{ATPV}/E_{BT}$ :  $40 \text{ cal}/\text{cm}^2$

Thus, NFPA 70E dictates the level of protection a fabric must possess to be worn by workers in certain environments.

NFPA 2112 (Standard on Flame-Resistant Clothing for Protection of Industrial Personnel Against Flash Fire, 2018 edition, incorporated herein by reference) governs the required performance of industrial worker garments that protect against flash fires. NFPA 1975 (Standard on Emergency Services Work Apparel, 2014 edition, incorporated herein by reference) governs the required performance of station wear worn by firefighter's in the firehouse and under turnout gear. NFPA 2112, ASTM F1506, and NFPA 1975 all require that the garments and/or individual layers or parts thereof pass a number of different performance tests, including compliance with the thermal protective requirements of having a char length of 4 inches or less (NFPA 2112) or 6 inches or less (ASTM F1506 and NFPA 1975) and of having a two second (or less) afterflame (NFPA 2112, ASTM F1506, and NFPA 1975), when measured pursuant to the testing methodology set forth in ASTM D6413 (Standard Test Method for Flame Resistance of Textiles, 2015 edition, incorporated herein by reference).

To test for char length and afterflame, a fabric specimen is suspended vertically over a flame for twelve seconds. The fabric must self-extinguish within two seconds (i.e., it must have a 2 second or less afterflame). After the fabric self-extinguishes, a specified amount of weight is attached to the fabric and the fabric lifted so that the weight is suspended from the fabric. The fabric will typically tear along the charred portion of the fabric. The length of the tear (i.e., the char length) must be 4 inches or less (ASTM 2112) or 6 inches or less (ASTM F1506 and NFPA 1975) when the test is performed in both the machine/warp and cross-machine/weft directions of the fabric. A fabric sample is typically tested for compliance both before it has been washed (and thus when the fabric still contains residual—and often flammable—chemicals from finishing processes) and after a certain number of launderings (e.g., 100 launderings for NFPA 2112 and 25 launderings for ASTM F1506).

NFPA 2112 and NFPA 1975 also contain requirements relating to the extent to which the fabric shrinks when subjected to heat. To conduct thermal shrinkage testing, marks are made on the fabric a distance from each other in both the machine/warp and cross-machine/weft directions. The distance between sets of marks is noted. The fabric is then suspended in a 500 degree Fahrenheit oven for 5 minutes. The distance between sets of marks is then re-measured. The thermal shrinkage of the fabric is then calculated as the percentage that the fabric shrinks in both the machine/warp and cross-machine/weft directions and must be less than the percentage set forth in the applicable standard. For example, NFPA 2112 and NFPA 1975 require that fabrics used in the construction of flame resistant garments exhibit thermal shrinkage of no more than 10% in both the machine/warp and cross-machine/weft directions.

NFPA 1975 further contains a thermal stability standard. To test for thermal stability, a fabric sample is folded and inserted between two glass plates. The sandwich is then put

in an oven at a specified temperature and for a specified time. After heating, the fabric is pulled apart. If the fabric sticks to itself, it fails the thermal stability test.

In the oil, gas, electric utility, and fire safety markets, there is a need for inexpensive, lightweight flame resistant fabrics that achieve a high arc rating while still complying with all applicable thermal protective requirements. More specifically, there is a need for inexpensive, lighter weight protective fabrics that achieve NFPA 70E PPE Category 2 protection (8 cal/cm<sup>2</sup> arc rating). Due to high temperature working conditions in some workplaces, end users also have a need for comfortable (e.g., breathable) protective fabrics that have excellent moisture management properties (e.g., wicking).

Historically, such fabrics have been formed from identical yarns made exclusively from cellulosic fibers treated with a chemical (e.g., phosphorous) to render them flame resistant. Cellulosic fibers are cheap, lightweight, and soft, thus rendering the fabrics into which they are incorporated inexpensive and comfortable. However, the flame resistance of these fibers is not inherent to the fibers themselves. Rather, the fibers must be chemically-treated to impart flame resistance to them. If the fibers are not treated properly, the chemicals can wash out of the fibers and thereby significantly diminish the flame resistant properties of the fibers and thus the fabrics and garments into which they are incorporated. Existing fabrics formed with inherently flame resistant fibers that do not suffer from this same drawback are more expensive and harsher to the touch. Thus, such fabrics have been unable to compete successfully in this space. There is a need for a comfortable, lightweight, inexpensive fabric formed with inherently flame resistant fibers that affords the requisite thermal and arc protection.

## SUMMARY

The terms “invention,” “the invention,” “this invention” and “the present invention” used in this patent are intended to refer broadly to all of the subject matter of this patent and the patent claims below. Statements containing these terms should not be understood to limit the subject matter described herein or to limit the meaning or scope of the patent claims below. Embodiments of the invention covered by this patent are defined by the claims below, not this summary. This summary is a high-level overview of various aspects of the invention and introduces some of the concepts that are further described in the Detailed Description section below. This summary is not intended to identify key or essential features of the claimed subject matter, nor is it intended to be used in isolation to determine the scope of the claimed subject matter. The subject matter should be understood by reference to the entire specification of this patent, all drawings and each claim.

Embodiments of the present invention relate to flame resistant fabrics formed with inherently flame resistant fibers that provide the requisite thermal and arc protection but that are less expensive than other fabrics formed with inherently flame resistant fibers and that have improved comfort. Improved comfort and lower cost can be achieved by predominantly locating the inherently flame resistant fibers on the front face of the fabric to impart the requisite thermal and arc protection and predominantly locating the more comfortable (and less expensive) fibers on the back face of the fabric positioned next to the wearer. In this way, overall protection of the fabric is maintained while improving comfort. Some embodiments of such fabrics may also achieve NFPA 70E PPE Category 2 protection ( $\geq 8$  cal/cm<sup>2</sup>

arc rating whether ATPV or EBT). Moreover, in some embodiments the flame resistant fabrics contain fibers having at least one energy absorbing and/or reflecting additive incorporated into the fibers. Inclusion of such fibers into the fabric increases the arc protection of the fabric while still complying with all requisite thermal protective requirements.

## DETAILED DESCRIPTION

The subject matter of embodiments of the present invention is described here with specificity to meet statutory requirements, but this description is not necessarily intended to limit the scope of the claims. The claimed subject matter may be embodied in other ways, may include different elements or steps, and may be used in conjunction with other existing or future technologies. This description should not be interpreted as implying any particular order or arrangement among or between various steps or elements except when the order of individual steps or arrangement of elements is explicitly described.

Some embodiments of the fabrics described herein have anisotropic properties in that the fabrics are constructed such that the body side of the fabric (the side of the fabric proximate the wearer (assuming the fabric will be incorporated into a garment)) and the face side of the fabric (the side of the fabric facing away from the wearer) have different properties. More specifically, in some embodiments a higher percentage of inherently flame resistant fibers (or yarns containing the fibers) are located and exposed on the face side of the fabric (as opposed to on the body side of the fabric). In such embodiments, a higher percentage of less expensive and more comfortable fibers (or yarns containing the fibers) are located and exposed on the body side of the fabric (as opposed to on the face side of the fabric). In such embodiments, the face side of the fabric thus effectively imparts the requisite thermal and arc protection and the body side of the fabric provides superior comfort and/or lower cost in relation to the face side of the fabric.

40 Fabrics according to such embodiments can be formed pursuant to any method that results in the fabric having different properties on the body side and the face side of the fabric. In some embodiments, the fabrics are a woven, knitted, and/or nonwoven fabric.

45 Woven and/or knitted fabrics may be formed to have anisotropic properties through the use of at least a first group of yarns and a second group of yarns, whereby each yarn group has a different fiber blend. The different fiber blends can be attributable to the two yarn groups having different amounts of the same fibers or to the two yarn groups having different fibers or different blends of fibers. In addition, it will be recognized that in some embodiments the yarns need not be blended at all. In other words, some yarns could be 100% of a single fiber type. Regardless, the first group of 50 yarns is predominantly exposed on the face side of the fabric and the second group of yarns is predominantly exposed on the body side of the fabric. In some embodiments, the fabric is formed only of the first group of yarns and the second group of yarns (i.e., these two yarn types form the entirety 55 of the fabric). In other embodiments, yarns in addition to the first and second groups of yarns may be incorporated into the fabric.

60 Fabrics of the invention may be formed with spun yarns, filament yarns, stretch broken yarns, or combinations thereof. The yarns can comprise a single yarn or two or more individual yarns that are combined together in some form, including, but not limited to, twisting, plying, tacking,

wrapping, covering, core-spinning (i.e., a filament or spun core at least partially surrounded by spun fibers or yarns), etc.

In some embodiments, the yarns of the first group of yarns ("first yarns") are spun yarns having a fiber blend that includes inherently flame resistant fibers. In some embodiments, the first yarns include at least 50% inherently flame resistant fibers, at least 55% inherently flame resistant fibers, at least 60% inherently flame resistant fibers, at least 65% inherently flame resistant fibers, at least 70% inherently flame resistant fibers, at least 75% inherently flame resistant fibers, at least 80% inherently flame resistant fibers, at least 85% inherently flame resistant fibers, and/or at least 90% inherently flame resistant fibers. Examples of suitable inherently flame resistant fibers include, but are not limited to, para-aramid fibers, meta-aramid fibers, polybenzoxazole ("PBO") fibers, polybenzimidazole ("PBI") fibers, modacrylic fibers, poly{2,6-diimidazo[4,5-b:40; 50-e]-pyridinylene-1,4(2,5-dihydroxy)phenylene} ("PIPD") fibers, polyacrylonitrile (PAN) fibers, liquid crystal polymer fibers, glass fibers, carbon fibers, TANLON™ fibers (available from Shanghai Tanlon Fiber Company), wool fibers, melamine fibers (such as BASOFIL™, available from Basofil Fibers), polyetherimide fibers, pre-oxidized acrylic fibers, polyamide-imide fibers such as KERMEL™, polytetrafluoroethylene fibers, polyetherimide fibers, polyimide fibers, and polyimide-amide fibers and any combination or blend thereof. Examples of para-aramid fibers include KEVLAR™ (available from DuPont), TECHNORA™ (available from Teijin Twaron BV of Arnheim, Netherlands), and TWARON™ (also available from Teijin Twaron By), and Taekwang para-aramid (available from Taekwang Industries). Examples of meta-aramid fibers include NOMEX™ (available from DuPont), CONEX™ (available from Teijin), APYEIL™ (available from Unitika), ARAWIN (available from Toray). An example of suitable modacrylic fibers are PROTEX™ fibers available from Kaneka Corporation of Osaka, Japan, SEFTM available from Solutia, or blends thereof.

The same inherently flame resistant fibers may be used in the first yarns, but such is not a requirement. Rather, the fiber blend of the first yarns may include the same type of inherently flame resistant fibers or, alternatively, different types of inherently flame resistant fibers may be provided in the blend.

In some embodiments, the inherently flame resistant fibers in the first yarns include a blend of aramid fibers (meta-aramid, para-aramid, or both) and modacrylic fibers. The modacrylic fibers are significantly less expensive than the aramid fibers, thus helping to contain the cost of the fabric. Moreover, in some embodiments the percentage of modacrylic fibers in the fiber blend of the first yarns is up to 2 times, up to 3 times, up to 4 times, up to 5 times, up to 6 times, up to 7 times, and/or up to 8 times the percentage of aramid fibers in the blend. In some embodiments, the first yarns include at least 40% modacrylic fibers, at least 45% modacrylic fibers, at least 50% modacrylic fibers, at least 55% modacrylic fibers, at least 60% modacrylic fibers, at least 65% modacrylic fibers, at least 70% modacrylic fibers, at least 75% modacrylic fibers, and/or at least 80% modacrylic fibers. In some embodiments, the first yarns include approximately (i) 40-90% modacrylic fibers, inclusive; (ii) 45-85% modacrylic fibers, inclusive; (iii) 50-80% modacrylic fibers, inclusive; (iv) 50-70% modacrylic fibers, inclusive; (v) 55-65% modacrylic fibers, inclusive; (vi) 60-80% modacrylic fibers, inclusive; and/or (vii) 65-75% modacrylic fibers, inclusive. In some embodiments, the first

yarns include at least 5% aramid fibers, at least 10% aramid fibers, at least 15% aramid fibers, at least 20% aramid fibers, at least 25% aramid fibers, at least 30% aramid fibers, and/or at least 35% aramid fibers. In some embodiments, the first

5 yarns include approximately (i) 5-35% aramid fibers, inclusive; (ii) 10-30% aramid fibers, inclusive; (iii) 15-25% aramid fibers, inclusive; (iv) 10-20% aramid fibers, inclusive; (v) 10-15% aramid fibers, inclusive; and/or (vi) 15-20% aramid fibers, inclusive.

10 In some embodiments, the first yarns include approximately (i) 5-35% aramid fibers and 40-90% modacrylic fibers, inclusive; (ii) 5-25% aramid fibers and 50-80% modacrylic fibers, inclusive; (iii) 10-20% aramid fibers and 50-80% modacrylic fibers, inclusive; (iv) 10-20% aramid fibers and 50-70% modacrylic fibers, inclusive; (v) 10-20% aramid fibers and 50-60% modacrylic fibers, inclusive; (vi) 15-25% aramid fibers and 60-80% modacrylic fibers, inclusive; (vii) 15-25% aramid fibers and 65-75% modacrylic fibers, inclusive; (viii) 18-23% aramid fibers and 65-75% modacrylic fibers, inclusive; (ix) 10-15% aramid fibers and 50-65% modacrylic fibers, inclusive; and/or (x) 10-15% aramid fibers and 50-60% modacrylic fibers, inclusive.

15 In some embodiments, cellulosic fibers may be added to the fiber blend of the first yarns to reduce cost and impart comfort. In some embodiments, the first yarns include at least 5% cellulosic fibers, at least 10% cellulosic fibers, at least 15% cellulosic fibers, at least 20% cellulosic fibers, at least 25% cellulosic fibers, at least 30% cellulosic fibers, at least 35% cellulosic fibers, at least 40% cellulosic fibers, at least 45% cellulosic fibers, or at least 50% cellulosic fibers. In some embodiments, the first yarns include approximately (i) 5-50% cellulosic fibers, inclusive; (ii) 10-35% cellulosic fibers, inclusive; (iii) 5-25% cellulosic fibers, inclusive; (iv) 30 5-20% cellulosic fibers, inclusive; (v) 5-15% cellulosic fibers, inclusive; (vi) 10-20% cellulosic fibers, inclusive; (vii) 10-15% cellulosic fibers, inclusive; (viii) 20-40% cellulosic fibers, inclusive; and/or (ix) 25-35% cellulosic fibers, inclusive.

35 40 In some embodiments, the cellulosic fibers are lyocell fibers and/or non-FR lyocell fibers. In some embodiments, blends of different cellulosic fibers are used in the fiber blend of the first yarns. While the cellulosic fibers can be treated so as to be flame resistant, this is not necessary. Rather,

45 50 inclusion of the inherently flame resistant fibers in the fiber blend imparts sufficient flame resistance and arc protection and prevents the cellulosic fibers from burning. For example, the modacrylic fibers control and counteract the flammability of the cellulosic fibers to prevent the cellulosic fibers from burning. In this way, the cellulosic fibers (or the yarns or fabrics made with such fibers) need not be treated with a FR compound or additive.

55 In some embodiments, the first yarns include approximately (i) 5-35% aramid fibers, 40-90% modacrylic fibers, and 5-50% cellulosic fibers (FR and/or non-FR), inclusive; (ii) 5-30% aramid fibers, 50-80% modacrylic fibers, and 10-40% cellulosic fibers (FR and/or non-FR), inclusive; (iii) 5-25% aramid fibers, 50-80% modacrylic fibers, and 15-40% cellulosic fibers (FR and/or non-FR), inclusive; (iv) 60 10-20% aramid fibers, 50-70% modacrylic fibers, and 20-45% cellulosic fibers (FR and/or non-FR), inclusive; (v) 10-20% aramid fibers, 50-70% modacrylic fibers, and 20-40% cellulosic fibers (FR and/or non-FR), inclusive; (vi) 10-15% aramid fibers, 55-70% modacrylic fibers, and 25-40% cellulosic fibers (FR and/or non-FR), inclusive; (vii) 10-30% aramid fibers, 60-80% modacrylic fibers, and 5-20% cellulosic fibers (FR and/or non-FR), inclusive; and/

or (viii) 15-25% aramid fibers, 65-75% modacrylic fibers, and 5-15% cellulosic fibers (FR and/or non-FR), inclusive.

In some embodiments, the yarns of the second group of yarns ("second yarns") are spun yarns having a fiber blend that includes more fibers that are more comfortable and less expensive than fibers in the first yarns. Such fibers include, but are not limited to, natural and synthetic cellulosic fibers (e.g., cotton, rayon, acetate, triacetate, and lyocell, as well as their flame resistant counterparts FR cotton, FR rayon, FR acetate, FR triacetate, and FR lyocell), modacrylic fibers, wool, TANLONTM fibers (available from Shanghai Tanlon Fiber Company), nylon fibers, polyester fibers, etc., and blends thereof. An example of FR rayon fibers is Lenzing FRTM fibers, also available from Lenzing Fibers Corporation, and VISILTM fibers, available from Sateri. Examples of lyocell fibers include TENCELTM, TENCEL G100TM and TENCEL A100TM fibers, all available from Lenzing Fibers Corporation. An example of a polyester fiber is DACRON® fibers (available from InvistaTM). Examples of suitable modacrylic fibers are PROTEXTM fibers available from Kaneka Corporation of Osaka, Japan, SEFTM fibers available from Solutia, PyroTex® fibers available from PyroTex Fibers GmbH, or blends thereof.

The second yarns preferably include cellulosic fibers for comfort, which can be FR and/or non-FR. In some embodiments, the cellulosic fibers are lyocell fibers and/or non-FR lyocell fibers. In some embodiments, the second yarns include at least 10% cellulosic fibers, at least 20% cellulosic fibers, at least 30% cellulosic fibers, at least 40% cellulosic fibers, at least 50% cellulosic fibers, at least 60% cellulosic fibers, at least 70% cellulosic fibers, at least 80% cellulosic fibers, or at least 90% cellulosic fibers. In some embodiments, the second yarns include approximately (i) 50-90% cellulosic fibers, inclusive; (ii) 55-85% cellulosic fibers, inclusive; (iii) 60-85% cellulosic fibers, inclusive; (iv) 65-85% cellulosic fibers, inclusive; (v) 70-85% cellulosic fibers, inclusive; (vi) 70-80% cellulosic fibers, inclusive; (vii) 60-75% cellulosic fibers, inclusive; and/or (viii) 65-75% cellulosic fibers, inclusive.

In some embodiments, the second yarns include a blend of cellulosic fibers and inherently flame resistant fibers (such as aramid fibers), which enhance thermal and arc protection and which help to resist thermal shrinkage. If inherently flame resistant fibers are included in the fiber blend of the second yarns, the percentage of such fibers are preferably (but do not have to be) less than the percentage of inherently flame resistant fibers used in the fiber blend of the first yarns. In some embodiments, inherently flame resistant fibers constitute 50% or less, 40% or less, 30% or less, or 20% or less of the fiber blend of the second yarns. In some embodiments, the second yarns include at least 10% inherently flame resistant fibers, at least 15% inherently flame resistant fibers, at least 20% inherently flame resistant fibers, at least 25% inherently flame resistant fibers, at least 30% inherently flame resistant fibers, at least 35% inherently flame resistant fibers, and/or at least 40% inherently flame resistant fibers. In some embodiments, the second yarns include approximately (i) 10-50% inherently flame resistant fibers, inclusive; (ii) 10-40% inherently flame resistant fibers, inclusive; (iii) 10-35% inherently flame resistant fibers, inclusive; (iv) 10-30% inherently flame resistant fibers, inclusive; (v) 15-25% inherently flame resistant fibers, inclusive; and/or (vi) 20-30% inherently flame resistant fibers, inclusive.

In some embodiments, the second group of yarns includes approximately (i) 50-90% cellulosic fibers and 10-50% inherently flame resistant fibers, inclusive; (ii) 60-90% cellulosic fibers and 10-40% inherently flame resistant fibers,

inclusive; (iii) 65-85% cellulosic fibers and 10-35% inherently flame resistant fibers, inclusive; (iv) 65-80% cellulosic fibers and 10-30% inherently flame resistant fibers, inclusive; (v) 70-80% cellulosic fibers and 20-30% inherently flame resistant fibers, inclusive; and/or (vi) 65-75% cellulosic fibers and 15-25% inherently flame resistant fibers, inclusive.

In some embodiments, different cellulosic fibers (e.g., blends of lyocell and rayon, blends of FR and non-FR cellulosic fibers, etc.) and/or inherently flame resistant fibers (e.g., para-aramid, meta-aramid, and/or modacrylic, etc.) are used in the fiber blend of the second yarns. In some embodiments, the inherently flame resistant fibers used in the fiber blend of the second yarns are modacrylic fibers and/or aramid fibers, such as para-aramid fibers, meta-aramid fibers, or blends thereof. In some embodiments, the modacrylic fibers constitute a greater percentage of the fiber blend of the second yarns than the aramid fibers. In some embodiments, the modacrylic fibers constitute 0-30% and the aramid fibers constitute 1-30% of the fiber blend of the second yarns. In some embodiments, the modacrylic fibers constitute 0-25% and the aramid fibers constitute 1-25% of the fiber blend of the second yarns. In some embodiments, the modacrylic fibers constitute 5-20% and the aramid fibers constitute 1-15% of the fiber blend of the second yarns. In some embodiments, the modacrylic fibers constitute 10-20% and the aramid fibers constitute 1-5% of the fiber blend of the second yarns. In some embodiments, the modacrylic fibers constitute 15-20% and the aramid fibers constitute 1-5% of the fiber blend of the second yarns.

In some embodiments, the second yarns include approximately (i) 1-20% aramid fibers, 5-40% modacrylic fibers, and 50-90% cellulosic fibers (FR and/or non-FR), inclusive; (ii) 1-15% aramid fibers, 10-35% modacrylic fibers, and 65-90% cellulosic fibers (FR and/or non-FR), inclusive; (iii) 1-10% aramid fibers, 10-25% modacrylic fibers, and 70-90% cellulosic fibers (FR and/or non-FR), inclusive; (iv) 1-5% aramid fibers, 10-20% modacrylic fibers, and 75-85% cellulosic fibers (FR and/or non-FR), inclusive; and/or (v) 1-5% aramid fibers, 15-20% modacrylic fibers, and 75-85% cellulosic fibers (FR and/or non-FR), inclusive.

In some embodiments, the fiber blend of the second yarns is devoid of modacrylic fibers. In some embodiments, aramid fibers are the only inherently flame resistant fibers provided in the second yarns. In such embodiments, the second yarns can include approximately (i) 5-50% aramid fibers, inclusive; (ii) 10-45% aramid fibers, inclusive; (iii) 10-40% aramid fibers, inclusive; (iv) 15-35% aramid fibers, inclusive; (v) 20-35% aramid fibers, inclusive; and/or (vi) 25-35% aramid fibers, inclusive.

In such embodiments, the second yarns include approximately (i) 50-90% cellulosic fibers and 10-50% aramid fibers, inclusive; (ii) 60-80% cellulosic fibers and 20-40% aramid fibers, inclusive; (iii) 65-80% cellulosic fibers and 25-35% aramid fibers, inclusive; and/or (iv) 65-75% cellulosic fibers and 25-35% aramid fibers, inclusive.

In some embodiments, the fiber blend of the overall fabric includes approximately (i) 25-65% cellulosic fibers (e.g., lyocell fibers and/or non-FR lyocell fibers), 25-65% modacrylic fibers, and 5-25% aramid fibers, inclusive; (ii) 30-60% cellulosic fibers (e.g., lyocell fibers and/or non-FR lyocell fibers), 25-60% modacrylic fibers, and 5-20% aramid fibers, inclusive; (iii) 35-60% cellulosic fibers (e.g., lyocell fibers and/or non-FR lyocell fibers), 30-55% modacrylic fibers, and 5-15% aramid fibers, inclusive; (iv) 40-60% cellulosic fibers (e.g., lyocell fibers and/or non-FR lyocell fibers), 30-50% modacrylic fibers, and 5-15% aramid fibers,

inclusive; (v) 40-55% cellulosic fibers (e.g., lyocell fibers and/or non-FR lyocell fibers), 30-50% modacrylic fibers, and 5-15% aramid fibers, inclusive; (vi) 45-55% cellulosic fibers (e.g., lyocell fibers and/or non-FR lyocell fibers), 35-45% modacrylic fibers, and 5-15% aramid fibers, inclusive; (vii) 25-50% cellulosic fibers (e.g., lyocell fibers and/or non-FR lyocell fibers), 25-50% modacrylic fibers, and 10-40% aramid fibers, inclusive; (viii) 30-45% cellulosic fibers (e.g., lyocell fibers and/or non-FR lyocell fibers), 30-45% modacrylic fibers, and 15-30% aramid fibers, inclusive; and/or (ix) 30-40% cellulosic fibers (e.g., lyocell fibers and/or non-FR lyocell fibers), 35-45% modacrylic fibers, and 20-30% aramid fibers, inclusive.

It may be beneficial, but not required, to include nylon fibers in either or both of the first yarns and the second yarns as nylon fibers impart abrasion resistance and thus enhance the durability and wear properties of the fabric made with such yarns.

It has also been discovered that incorporating into the fabric (via the first yarns, second yarns, or otherwise) fibers having at least one energy absorbing and/or reflecting additive increases the arc rating of the fabric while still complying with all requisite thermal protective requirements.

It is believed that such energy (e.g., radiation) absorbing and/or reflecting additives serve to prevent heat energy transmission through the fabric and to the wearer's skin by absorbing the energy and/or reflecting the energy away from the fabric such that it does not reach the wearer. Additive-containing fibers ("AC fibers") are fibers whereby an energy absorbing and/or reflecting additive is introduced during the process of manufacturing the fibers themselves and not after fiber formation. This is in contrast to a finish applied onto the fabric surface whereby a binder typically must be used to fix the additive onto the fabric. In these cases, the additive is apt to wash and/or wear/abrade off the fabric during laundering. Provision of the additive in the fibers during fiber formation results in better durability as the additive is trapped within the fiber structure. Examples of AC fibers are identified and described in U.S. Patent Publication No. 2017/0370032 to Stanhope et al., U.S. Patent Publication No. 2017/0295875 to Ohzeki et al., and U.S. patent Ser. No. 16/271,162 to Stanhope et al., the entirety of each of which is herein incorporated by reference. Note that while AC fibers may be used in embodiments of the fabrics contemplated herein, they need not always be used. For example, some AC fibers are producer-colored fibers. In producer coloring (also known as "solution dyeing"), pigment is injected into the polymer solution prior to forming the fibers. Thus, "producer-colored" fibers refers to fibers that are colored during the process of manufacturing the fibers themselves and not after fiber formation. If darker-colored additives (such as navy and black) are used to color the fibers, use of such darker fibers (such as producer-colored aramid fibers) in fabrics may render the fabrics more difficult to dye to lighter shades of color. Thus, it might not always be desirable to use AC aramid fibers in the blends disclosed herein, particularly if such AC aramid fibers are darker shades.

If AC fibers are desired, the AC fibers may be incorporated into either or both of the first and second yarns. In some embodiments, the AC fibers are incorporated into the first yarns so as to be exposed on the face side of the fabric. For example, in some embodiments the AC fibers are modacrylic fibers that include an infrared absorber, such as described in U.S. Patent Publication No. 2017/0295875 to Ohzeki et al. and/or sold as PROTEX<sup>TM</sup> A fibers by Kaneka Corporation of Osaka, Japan (as opposed to PROTEX<sup>TM</sup> C fibers which do not contain such an additive).

In some embodiments, the AC fibers are incorporated into the fiber blend of the first yarns to enhance the arc protection on the face of the fabric. In some embodiments, the AC fibers are only incorporated into the fiber blend of the first 5 yarns and are not incorporated into the second yarns. In some embodiments, the modacrylic fibers in the first yarns are AC fibers, such as, but not limited to, PROTEX<sup>TM</sup> A fibers.

The AC fibers provided in the fabric need not all be the 10 same. For example, the fiber blend may include the same type of AC fiber or, alternatively, different types of AC fibers may be provided in the blend.

In some embodiments, the AC fibers (such as the AC 15 version of any of the fibers identified above) constitute 20-60%, inclusive, of the fiber blend of the fabric; 20-50%, inclusive, of the fiber blend of the fabric; 25-50%, inclusive, of the fiber blend of the fabric; 25-45%, inclusive, of the fiber 20 blend of the fabric; 30-45%, inclusive, of the fiber blend of the fabric; or 35-45%, inclusive, of the fiber blend of the fabric. In some embodiments, the AC fibers constitute 25 at least 5% or at least 10% or at least 15% or at least 20% or at least 25% or at least 30% or at least 35% or at least 40% or at least 45% and (i) no more than 60%, (ii) no more than 50%, (iii) no more than 45%, (iv) no more than 40%, or (v) no more than 35%, inclusive, of the fiber blend of the fabric.

In some embodiments, the fabrics are woven fabrics 30 formed of the first yarns and the second yarns. In some embodiments, only the first yarns will be oriented in the warp direction and only the second yarns will be oriented in the fill direction. In this way, the fibers on the face side of the fabric will predominantly comprise those of the first yarns and the fibers on the body side of the fabric will predominantly comprise those of the second yarns.

In other embodiments, not all of the warp or fill yarns are 35 the same. For example, the first and second yarns may be provided in both the warp and fill directions by providing the first yarns on some ends and picks and the second yarns on other ends and picks (in any sort of random arrangement or alternating pattern). Or all of the yarns in one of the warp or 40 fill direction could be identical (e.g., either all first yarns or all second yarns) and different yarns (both first and second yarns) used only in the other of the warp or fill direction.

The fabric may be constructed with the first and second 45 yarns in a variety of ways, including but not limited to, one or more of twill weave (2x1, 3x1, etc.), twill weave containing a rip-stop pattern, satin weave (4x1, 5x1, etc.), sateen weave, and double-cloth constructions, or any other weave where yarn is predominantly more on one side of the fabric than the other side of the fabric. A person skilled in the 50 art would be familiar with and could utilize suitable fabric constructions.

It will also be recognized that any woven fabric will have both warp and fill yarns visible on each side of the fabric. Fabrics woven in accordance with some embodiments of the 55 present invention, however, are woven such that more of the first yarns are located on the face side of the fabric, and thus more of the second yarns are located on the body side of the fabric. Thus, in an exemplary fabric construction in which more of the first yarns are located or exposed on the face side 60 of the fabric and more of the second yarns are located or exposed on the body side of the fabric, the first yarns are "predominantly" exposed on the face side of the fabric (even though some of the first yarns would be visible from the body side of the fabric) and the second yarns are "predominantly" exposed on the body side of the fabric (even though some of the second yarns would be visible from the face side 65 of the fabric).

## 11

In other embodiments of the invention, a knit fabric that has different properties on each side of the fabric can be constructed. Such a fabric could be constructed using double-knit technology such that the first yarns will be predominantly exposed on the face side of the fabric and the second yarns will be predominantly exposed on the opposing body side of the fabric.

Embodiments of the fabric can be of any weight, but in some embodiments are between 5 to 7 ounces per square yard (osy), inclusive. In some embodiments, the fabric weight is at least 5 osy but less than or equal to 7 osy, 6.9 osy, 6.8 osy, 6.7 osy, 6.6 osy, 6.5 osy, 6.4 osy, 6.3 osy, 6.2 osy, 6.1 osy, 6.0 osy, 5.9 osy, 5.8 osy, 5.7 osy, 5.6 osy, 5.5 osy, 5.4 osy, 5.3 osy, 5.2 osy, and/or 5.1 osy.

Fabrics according to some embodiments of the present invention strategically place fibers useful for thermal and arc protection (e.g., aramid fibers which tend to be more expensive and less comfortable) on the face side of the fabric and more comfortable, less expensive fibers on the body side of the fabric. These fabrics thus provide the requisite protection to the wearer while rendering the garment more comfortable

## 12

and affordable as compared to existing fabrics. The cost of the fabrics is contained due to (among other things): (1) incorporation of cellulosic fibers in the first yarns and inclusion of large amounts of cellulosic fibers in the second 5 yarns; (2) limiting the amount of inherently FR fibers (more expensive fibers such as aramid fibers) in the fabric but concentrating those fibers on the face of the fabric; (3) inclusion of inherently FR fibers, which permits lower 10 weight (and thus less expensive) fabrics to perform as required; (4) use of more modacrylic fibers than aramid fibers, which are significantly less expensive while still imparting thermal and arc protection to the fabric; and/or (5) use of AC fibers in the first yarns so as to be predominantly 15 exposed on the face side of the fabric where the AC fibers are more effective for improving ATPV than if they were exposed on the body side of the fabric.

Table 1 sets forth testing results of various properties of some embodiments of the inventive fabrics contemplated herein (Fabrics 1-5). Fabrics 1-5 were finished but without 20 the use of any property-imparting (e.g., flame retardant) additive.

TABLE 1

| Property                                 | Fabric 1                                          | Fabric 2                                           | Fabric 3                                          | Fabric 4                                           | Fabric 5                                            |                                       |
|------------------------------------------|---------------------------------------------------|----------------------------------------------------|---------------------------------------------------|----------------------------------------------------|-----------------------------------------------------|---------------------------------------|
| First Yarn Blend                         | 55 Protex<br>A/35<br>Tencel/<br>5 Meta/<br>5 Para | 55 Protex<br>A/30<br>Tencel/<br>10 Meta/<br>5 Para | 60 Protex<br>A/25<br>Tencel/<br>7 Meta/<br>5 Para | 60 Protex<br>A/28<br>Tencel/<br>10 Meta/<br>5 Para | 70 Protex<br>A/10<br>Tencel/<br>10 Meta/<br>10 Para |                                       |
| Second Yarn Blend                        | 80 Tencel/<br>17 Protex<br>C/3 Para               | 80 Tencel/<br>17 Protex<br>C/3 Para                | 80 Tencel/<br>17 Protex<br>C/3 Para               | 80 Tencel/<br>17 Protex<br>C/3 Para                | 70 Tencel/<br>25 Meta/<br>5 Para                    | NFPA 70E/<br>ASTM 1506<br>Requirement |
| Weave                                    | 2 x 1 RHT                                         | 2 x 1 RHT                                          | 2 x 1 RHT                                         | 2 x 1 RHT                                          | 2 x 1 RHT                                           | NFPA 2112<br>Requirement              |
| Width Overall (in)                       | 61.8                                              | 62.2375                                            | 61.075                                            | 62.25                                              | 62.275                                              |                                       |
| Width Inside Pins (in)                   | 60.98                                             | 61.06                                              | 60.48                                             | 61.28                                              | 61.36                                               |                                       |
| Weight (osy)                             | 6                                                 | 5.9                                                | 5.9                                               | 5.8                                                | 5.7                                                 |                                       |
| Construction (w x f)                     | 64 x 52                                           | 64 x 50                                            | 65 x 50                                           | 65 x 50                                            | 76 x 56                                             |                                       |
| Vertical                                 |                                                   |                                                    |                                                   |                                                    |                                                     |                                       |
| Flammability - Before Wash               |                                                   |                                                    |                                                   |                                                    |                                                     |                                       |
| After Flame (sec)                        | 0 x 0                                             | 0 x 0                                              | 0 x 0                                             | 0 x 0                                              | 0 x 0                                               | <2 x 2                                |
| Char Length (inch)                       | 3.4 x 2.9                                         | 3.5 x 2.5                                          | 3.6 x 2.5                                         | 3.6 x 2.9                                          | 2.0 x 2.9                                           | <6 x 6                                |
| After Glow (sec)                         | 3 x 3                                             | 2 x 2                                              | 2 x 2                                             | 2 x 2                                              | 2 x 2                                               | <4 x 4                                |
| Vertical                                 |                                                   |                                                    |                                                   |                                                    |                                                     |                                       |
| Flammability - After 100x IL*            |                                                   |                                                    |                                                   |                                                    |                                                     |                                       |
| After Flame (sec)                        | 0 x 0                                             | 0 x 0                                              | 0 x 0                                             | 0 x 0                                              | 0 x 0                                               | <2 x 2                                |
| Char Length (inch)                       | 3.4 x 3.4                                         | 3.5 x 2.2                                          | 3.9 x 2.2                                         | 3.3 x 2.6                                          | 2.0 x 3.3                                           | <4 x 4                                |
| After Glow (sec)                         | 8 x 7                                             | 7 x 6                                              | 7 x 7                                             | 7 x 7                                              | 5 x 6                                               |                                       |
| Tensile Strength (lbf)                   | 99 x 93                                           | 107 x 79                                           | 114 x 96                                          | 112 x 91                                           | 110 x 95                                            | 30 x 30                               |
| Elmendorf Tear (lbf)                     | 9.8 x 10                                          | 11.5 x 10.4                                        | 12.0 x 10.2                                       | 10.8 x 10.5                                        | 8.6 x 7.7                                           | 2.5 x 2.5                             |
| Laundry Shrinkage (%) - After 5x PP120** | -5.3 x -6.5                                       | -4.0 x -6.4                                        | -4.2 x -5.4                                       | -4.2 x -6.5                                        | -3.0 x -1.8                                         |                                       |
| Thermal Shrinkage (%)                    |                                                   |                                                    |                                                   |                                                    |                                                     |                                       |
| Before Wash                              | -8.4 x -4.3                                       | -7.1 x -4.8                                        | -8.1 x -5.3                                       | -8.3 x -5.5                                        | -7.1 x -2.6                                         | <10 x 10                              |
| After 3x IL                              | -8.2 x -5.3                                       | -6.1 x -5.2                                        | -7.5 x -5.1                                       | -7.4 x -5.2                                        | -5.4 x -3.0                                         | <10 x 10                              |
| Air permeability (cfm/ft <sup>2</sup> )  | 144                                               | 161                                                | 142                                               | 154                                                | 99                                                  |                                       |
| HTP - Before Wash (cal/cm <sup>2</sup> ) |                                                   |                                                    |                                                   |                                                    |                                                     |                                       |
| with Spacer                              | 10.3                                              | 10.2                                               | 10.3                                              | 10.3                                               | 9.8                                                 | >6                                    |
| w/o Spacer                               | 7.3                                               | 7.3                                                | 7.1                                               | 7.2                                                | 6.8                                                 | >3                                    |

TABLE 1-continued

| Property                                             | Fabric 1 | Fabric 2 | Fabric 3 | Fabric 4 | Fabric 5 |    |
|------------------------------------------------------|----------|----------|----------|----------|----------|----|
| <u>HTP-<br/>After 3x IL<br/>(cal/cm<sup>2</sup>)</u> |          |          |          |          |          |    |
| with Spacer                                          | 12.3     | 12       | 11.4     | 11.8     | 11       | >6 |
| w/o Spacer                                           | 8.7      | 8.1      | 8.2      | 8.6      | 7.6      | >3 |
| Wicking Droplet<br>Test (s)                          |          |          |          |          |          |    |
| Before Wash                                          | 0.5      | 0.5      | 0.4      | 0.4      | 0.7      |    |
| After 5x PP120                                       | 0.8      | 0.9      | 0.9      | 1        | 2.5      |    |
| Arc Rating<br>(cal/cm <sup>2</sup> )                 | 8        | 8.6      | 8.1      | 8.3      | 8.5      |    |

\*The fabrics were laundered in accordance with the industrial laundering (“IL”) specifications set forth in NFPA 2112.

\*\*The fabrics were laundered in accordance with AATCC Method 135, 3, IV, A iii (*Dimensional Changes of Fabrics after Home Laundering*, 2018 edition, incorporated herein by reference). More specifically, the fabrics were laundered via permanent press at 120° F. (“PP120”).

Vertical flammability (char length, after flame, and after glow) were tested in accordance with ASTM D6413: *Standard Test Method for Flame Resistance of Textiles (Vertical Test)* (2015 edition). Tensile strength was tested in accordance with D5034: *Standard Test Method for Breaking Strength and Elongation of Textile Fabrics (Grab Test)* (2009 edition), and the results are represented in pounds force (“lbf”). Elmendorf tear strength was tested in accordance with ASTM D1424: *Standard Test Method for Tearing Strength of Fabrics by Falling-Pendulum (Elmendorf-Type) Apparatus* (2009 edition), and the results are represented in pounds force (“lbf”). Laundry shrinkage was tested in accordance with AATCC Method 135, 3, IV, A iii: *Dimensional Changes of Fabrics after Home Laundering* (2018 edition). Thermal shrinkage was tested in accordance with NFPA 2112. Heat transfer performance/radiant heat resistance (“HTP”) was tested in accordance with ASTM F1939: *Standard Test Method for Radiant Heat Resistance of Flame Resistant Clothing Materials with Continuous Heating* (2015 edition), and the results are reported in calories per centimeter<sup>2</sup>. All of these testing methodologies are incorporated herein by reference.

Embodiments of the fabrics disclosed herein comply with the vertical flammability requirements of both ASTM F1506 (char length of 6 inches or less and a two second or less afterflame) and NFPA 2112 (char length of 4 inches or less and a two second or less afterflame), when measured pursuant to the testing methodology set forth in ASTM D6413, as well as the thermal shrinkage requirement (no more than 10% thermal shrinkage) of NFPA 2112.

Moreover, many of the inventive fabrics achieved an arc rating (ATPV or E<sub>BT</sub>) greater or equal to 8 cal/cm<sup>2</sup> so as to have a PPE Category 2 rating under NFPA 70E even at low weights (e.g., between 5-7 osy, inclusive). Embodiments of the fabrics disclosed herein achieve surprisingly high arc rating/fabric weight ratios. In some embodiments, the arc rating/fabric weight ratio is 1.1-1.6, inclusive; 1.2-1.6, inclusive; 1.3-1.6, inclusive; 1.4-1.6, inclusive; and 1.4-1.5, inclusive. In some embodiments, the arc rating/fabric weight ratio is at least 1.2; at least 1.25; at least 1.3; at least 1.35; at least 1.4; at least 1.45; at least 1.5; at least 1.55; and/or at least 1.6. Even higher arc rating/fabric weight ratios may be achieved by increasing the amount of AC fibers (FR or non-FR) in the blend.

Incorporation of cellulosic and modacrylic fibers in the fiber blends impart excellent moisture management properties to the fabric when tested pursuant to AATCC 79: *Absorbency of Textiles* (2018 edition, incorporated herein by

reference). In other words, the fabrics are able to quickly draw moisture away from the wearer’s body via capillary action. Under AATCC 79, a droplet of water is deposited on the fabric surface, and the time it takes for the droplet to absorb fully into the fabric is measured. Some embodiments of the fabrics contemplated herein achieve an absorbency time of 5 seconds or less when tested pursuant to AATCC 79, as evidenced in Tables 1-4 (see “Wicking Droplet Test”). Such testing is to be performed on unfinished fabrics as the wicking property of a fabric can be easily manipulated with the use of finishes.

In addition to wicking ability, the air permeability of the fabric is also relevant to the comfort of the fabric. The air permeability of a fabric is determined by test method ASTM D737: *Standard Test Method for Air Permeability of Textile Fabrics* (2018 edition, incorporated herein by reference) and gauges how easily air passes through a fabric. The fabric is placed on a device that blows air through the fabric, and the device measures the volume flow of air through the fabric at a particular pressure (reported as “f<sup>3</sup>/min/ft<sup>2</sup>” or cubic foot per minute per square foot). Higher air permeability values mean that the fabric is more breathable, which is typically desirable. Embodiments of the fabric contemplated herein have good air permeability (in the range of 80-250 f<sup>3</sup>/min/ft<sup>2</sup>, inclusive; 90-200 f<sup>3</sup>/min/ft<sup>2</sup>, inclusive; 100-150 f<sup>3</sup>/min/ft<sup>2</sup>, inclusive) when tested pursuant to ASTM D737.

The fabrics described herein can be incorporated into any type of single or multi-layer garment (uniforms, shirts, jackets, trousers and coveralls) where protection against electric arc flash and/or flames is needed and/or desirable.

## EXAMPLES

A collection of exemplary embodiments, including at least some explicitly enumerated as “Examples” providing additional description of a variety of example types in accordance with the concepts described herein are provided below. These examples are not meant to be mutually exclusive, exhaustive, or restrictive; and the invention is not limited to these example examples but rather encompasses all possible modifications and variations within the scope of the issued claims and their equivalents.

Example 1. A fabric formed by first yarns and a second yarns, wherein the fabric has a first side and a second side opposite the first side and wherein: the first yarns comprise a first fiber blend comprising aramid fibers, modacrylic fibers, and cellulosic fibers; the aramid fibers and the modacrylic fibers of the first fiber blend constitute at least

50% of the first fiber blend; the first fiber blend comprises more modacrylic fibers than aramid fibers; the second yarns comprises a second fiber blend that is different from the first fiber blend and that comprises aramid fibers, modacrylic fibers, and cellulosic fibers; the second fiber blend comprises at least 60% cellulosic fibers; the second fiber blend comprises more modacrylic fibers than aramid fibers; the first yarns are predominantly exposed on the first side of the fabric; the second yarns are predominantly exposed on the second side of the fabric; the fabric has a char length of at least 6 inches and an afterflame of 2 seconds or less when tested pursuant to ASTM D6413 (2015); the fabric has a fabric weight between 5 to 7 ounces per square yard, inclusive; and the fabric has an arc rating of at least 8 cal/cm<sup>2</sup> when tested pursuant to ASTM F1959 (2014).

Example 2. The fabric of any of the preceding or subsequent examples or combination of examples, wherein the aramid fibers and the modacrylic fibers of the first fiber blend constitute at least 60% of the first fiber blend.

Example 3. The fabric of any of the preceding or subsequent examples or combination of examples, wherein the first fiber blend comprises up to 2 times more modacrylic fibers than aramid fibers.

Example 4. The fabric of any of the preceding or subsequent examples or combination of examples, wherein the first fiber blend comprises up to 3 times more modacrylic fibers than aramid fibers.

Example 5. The fabric of any of the preceding or subsequent examples or combination of examples, wherein the first fiber blend comprises approximately 5-25% aramid fibers, 50-80% modacrylic fibers, and 15-40% cellulosic fibers.

Example 6. The fabric of any of the preceding or subsequent examples or combination of examples, wherein the cellulosic fibers in the first fiber blend are non-FR lyocell fibers.

Example 7. The fabric of any of the preceding or subsequent examples or combination of examples, wherein the modacrylic fibers in the first fiber blend are additive-containing fibers.

Example 8. The fabric of any of the preceding or subsequent examples or combination of examples, wherein the aramid fibers in the first fiber blend comprise meta-aramid fibers and para-aramid fibers.

Example 9. The fabric of any of the preceding or subsequent examples or combination of examples, wherein the second fiber blend comprises at least 70% cellulosic fibers.

Example 10. The fabric of any of the preceding or subsequent examples or combination of examples, wherein the modacrylic fibers and aramid fibers of the second fiber blend constitute 40% or less of the second fiber blend.

Example 11. The fabric of any of the preceding or subsequent examples or combination of examples, wherein the fabric is a woven fabric comprising a first fabric direction and a second fabric direction opposite the first fabric direction, wherein the first yarns are provided only in the first fabric direction and the second yarns are provided only in the second fabric direction.

Example 12. A garment formed with the fabric of any of the preceding or subsequent examples or combination of examples, the garment having a face side and a body side, wherein the first side of the fabric is exposed on the face side of the garment and the second side of the fabric is exposed on the body side of the garment.

Example 13. A fabric formed by first yarns and a second yarns, wherein the fabric has a first side and a second side opposite the first side and wherein: the first yarns comprise

a first fiber blend comprising aramid fibers, modacrylic fibers, and cellulosic fibers; the aramid fibers and the modacrylic fibers of the first fiber blend constitute at least 70% of the first fiber blend; the first fiber blend comprises more modacrylic fibers than aramid fibers; the second yarns comprises a second fiber blend that is different from the first fiber blend and that comprises aramid fibers and non-FR cellulosic fibers; the second fiber blend is devoid of modacrylic fibers; the second fiber blend comprises at least 50% non-FR cellulosic fibers; the first yarns are predominantly exposed on the first side of the fabric; the second yarns are predominantly exposed on the second side of the fabric; the fabric has a char length of at least 6 inches and an afterflame of 2 seconds or less when tested pursuant to ASTM D6413 (2015); the fabric has a fabric weight between 5 to 7 ounces per square yard, inclusive; and the fabric has an arc rating of at least 8 cal/cm<sup>2</sup> when tested pursuant to ASTM F1959 (2014).

Example 14. The fabric of any of the preceding or subsequent examples or combination of examples, wherein the aramid fibers and the modacrylic fibers of the first fiber blend constitute at least 80% of the first fiber blend.

Example 15. The fabric of any of the preceding or subsequent examples or combination of examples, wherein the first fiber blend comprises up to 3 times more modacrylic fibers than aramid fibers.

Example 16. The fabric of any of the preceding or subsequent examples or combination of examples, wherein the first fiber blend comprises approximately 5-30% aramid fibers, 50-80% modacrylic fibers, and 10-40% cellulosic fibers.

Example 17. The fabric of any of the preceding or subsequent examples or combination of examples, wherein the second fiber blend comprises at least 60% non-FR cellulosic fibers.

Example 18. The fabric of any of the preceding or subsequent examples or combination of examples, wherein the aramid fibers of the second fiber blend constitute 40% or less of the second fiber blend.

Example 19. The fabric of any of the preceding or subsequent examples or combination of examples, wherein the fabric is a woven fabric comprising a first fabric direction and a second fabric direction opposite the first fabric direction, wherein the first yarns are provided only in the first fabric direction and the second yarns are provided only in the second fabric direction.

Example 20. A garment formed with the fabric of any of the preceding or subsequent examples or combination of examples, the garment having a face side and a body side, wherein the first side of the fabric is exposed on the face side of the garment and the second side of the fabric is exposed on the body side of the garment.

Different arrangements of the components described above, as well as components and steps not shown or described are possible. Similarly, some features and sub-combinations are useful and may be employed without reference to other features and subcombinations. Embodiments of the invention have been described for illustrative and not restrictive purposes, and alternative embodiments will become apparent to readers of this patent. Accordingly, the present invention is not limited to the embodiments described above or depicted in the drawings, and various embodiments and modifications can be made without departing from the scope of the invention.

We claim:

1. A fabric formed by first yarns and second yarns, wherein the fabric has a first fabric side and a second fabric side opposite the first fabric side and wherein:
  - i. the first yarns comprise a first fiber blend comprising aramid fibers, modacrylic fibers, and 5-15% cellulosic fibers;
  - ii. the aramid fibers and the modacrylic fibers of the first fiber blend constitute at least 70% of the first fiber blend;
  - iii. the first fiber blend comprises more modacrylic fibers than aramid fibers;
  - iv. the second yarns comprise a second fiber blend that is different from the first fiber blend and that comprises aramid fibers and non-FR cellulosic fibers;
  - v. the second fiber blend is devoid of modacrylic fibers;
  - vi. the second fiber blend comprises at least 50% non-FR cellulosic fibers;
  - vii. the first yarns are predominantly exposed on the first fabric side;
  - viii. the second yarns are predominantly exposed on the second fabric side;
  - ix. the fabric has a char length of 6 inches or less and an afterflame of 2 seconds or less when tested pursuant to ASTM D6413 (2015);
  - x. the fabric has a fabric weight between 5 to 7 ounces per square yard, inclusive; and
  - xi. the fabric has an arc rating of at least 8 cal/cm<sup>2</sup> when tested pursuant to ASTM F1959 (2014).
2. The fabric of claim 1, wherein the aramid fibers and the modacrylic fibers of the first fiber blend constitute at least 80% of the first fiber blend.
3. The fabric of claim 1, wherein the first fiber blend comprises up to 3 times more modacrylic fibers than aramid fibers.
4. The fabric of claim 1, wherein the first fiber blend comprises approximately 5-30% aramid fibers, 50-80% modacrylic fibers, and 10-15% cellulosic fibers.
5. The fabric of claim 1, wherein the second fiber blend comprises at least 60% non-FR cellulosic fibers.
6. The fabric of claim 1, wherein the aramid fibers of the second fiber blend constitute 40% or less of the second fiber blend.

7. The fabric of claim 1, wherein the fabric is a woven fabric comprising a first fabric direction and a second fabric direction opposite the first fabric direction, wherein the first yarns are provided only in the first fabric direction and the second yarns are provided only in the second fabric direction.
8. A garment formed with the fabric of claim 1 and having a face side and a body side, wherein the first fabric side is exposed on the face side of the garment and the second fabric side is exposed on the body side of the garment.
9. A fabric formed by first yarns and second yarns and comprising a first fabric direction, a second fabric direction opposite the first fabric direction, a first fabric side, and a second fabric side opposite the first fabric side, wherein:
  - i. the first yarns comprise a first fiber blend comprising approximately 5-30% aramid fibers, 50-80% modacrylic fibers, and 5-15% cellulosic fibers;
  - ii. the aramid fibers and the modacrylic fibers of the first fiber blend constitute at least 70% of the first fiber blend;
  - iii. the first fiber blend comprises more modacrylic fibers than aramid fibers;
  - iv. the second yarns comprises a second fiber blend that is different from the first fiber blend and that comprises aramid fibers and non-FR cellulosic fibers;
  - v. the second fiber blend is devoid of modacrylic fibers;
  - vi. the second fiber blend comprises at least 50% non-FR cellulosic fibers;
  - vii. the aramid fibers of the second fiber blend constitute 40% or less of the second fiber blend;
  - viii. the first yarns are predominantly exposed on the first fabric side and the second yarns are predominantly exposed on the second fabric side;
  - ix. the first yarns are provided only in the first fabric direction and the second yarns are provided only in the second fabric direction;
  - x. the fabric has a char length of 6 inches or less and an afterflame of 2 seconds or less when tested pursuant to ASTM D6413 (2015);
  - xi. the fabric has a fabric weight between 5 to 7 ounces per square yard, inclusive; and
  - xii. the fabric has an arc rating of at least 8 cal/cm<sup>2</sup> when tested pursuant to ASTM F1959 (2014).

\* \* \* \* \*